

## UNITED STATES PATENT OFFICE

2,191,731

## STENCIL SHEET

Walter O. Snelling, Allentown, Pa., assignor to  
Trojan Powder Company, Allentown, Pa.

No Drawing. Application July 2, 1938,  
Serial No. 217,308

3 Claims. (Cl. 41—38.6)

My invention relates to improvements in stencil sheets, and more particularly relates to improved stencil sheets of the so-called "indestructible" type, for use in the preparation of large numbers of copies closely simulating typewritten matter.

Stencil sheets for use on a typewriter or for use with a stylus for purposes of reduplication of typewritten matter or other desired symbols have been used for many years. The earliest stencil sheets adapted to use with a typewriter were of a wax base, and these were followed by stencil sheets of a protein base, but the discovery of the cellulose ester type of stencil sheet, as described in U. S. Patent 1,526,982 of February 17th, 1925, to Edward H. Hill, represented a great improvement in the art of stencil sheet manufacture, and my present invention represents an improvement in stencil sheets of this general type.

I have discovered that the substitution of nitrocellulose by nitrostarch in the preparation of stencils of the cellulose ester type leads to greatly improved results, and affords the means of preparing stencil sheets that represent a marked improvement over any of the types of stencil sheets known up to this time.

In order to explain why the substitution of nitrocellulose by nitrostarch leads to such marked improvement in stencil sheets, and in order to explain the greatly improved results that are obtained with nitrostarch stencil sheets as compared with nitrocellulose stencil sheets, it is necessary to describe some of the physical characteristics of nitrocellulose or cellulose nitrate. Cellulose nitrate is a material characterized by relatively great tensile strength and extreme toughness, and when cellulose nitrate is dissolved in a solvent, and the solvent is evaporated to leave a film of residual cellulose nitrate, the cellulose nitrate film thus formed is normally very strong and very tough. It may be "loaded" with considerable amounts of oils, waxes, resins and inert diluents, while still retaining a considerable measure of its normal strength and toughness.

I have discovered that when nitrostarch is substituted for nitrocellulose in this type of coating compositions which is used for stencil sheets, using the identical formulas used with the nitrocellulose compositions, the film of nitrostarch in admixture with the tempering agents that is left on the porous paper is relatively weak and friable (type-rupturable), as compared with the corresponding film left after the evaporation of solvents from a corresponding nitrocellulose so-

lution. This increased friability of the nitrostarch assists in the ready pulverization or disintegration of the film from the impact of the type key, and the lack of tensile strength of the nitrostarch film enables the coating on the porous backing paper to be more readily perforated and removed by the action of the impact of the type key than is possible when nitrocellulose is used in the coating composition, while the brittleness of the nitrostarch film facilitates the complete breaking up of the film at the point of impact, and the non-adherence of the disintegrated particles of the nitrostarch film greatly assists in promoting the openness and porosity of the prepared stencil at the points through which the duplicating ink is to be forced, in the subsequent operation of the stencil.

I have discovered that although nitrostarch has all the advantages of nitrocellulose in affording a film on porous paper that is normally impermeable to greasy inks at points where the coherence and continuity of the film has not been interrupted by impact with a type key or attrition or pressure from a stylus or the like, it has great advantages over corresponding films of a cellulose ester base because of the much clearer nature of the prints that it produces, this greater clearness of the prints being due to the fact that the low tensile strength of the nitrostarch film, and its decided friability under the influence of impact or pressure, and the almost entire lack of coherence of the finely comminuted material that is produced when the film is broken by impact, friction, attrition or pressure, all lead to the production of increased openness and "cleanliness" of the work of the finished stencil.

This increased openness of the portions of the stencil subjected to impact of the keys is not gained at the cost of greater porosity of the original sheet, and I have found that the original nitrostarch coating before impact or preparation with a stylus or the like is just as non-permeable to the duplicating ink as a similar stencil sheet of nitrocellulose base. It is only after preparation by impact or the like that the friable and readily disintegrated nature of the deposited nitrostarch film shows the characteristic of high permeability to the duplicating ink, and accordingly the original porous sheet coated with nitrostarch stencil composition is not any more porous to an oily or greasy duplicating ink than is a nitrocellulose sheet of corresponding composition, but after preparation in a typewriter, the nitrostarch sheet shows much better printing or duplicating properties than a nitrocellulose sheet.

The advantages which my porous stencil sheets coated with nitrostarch coating compositions have over sheets of exactly similar porous paper coated with corresponding nitrocellulose coating compositions as shown in the earlier art, are not alone to be found in the increased clearness of the duplicated matter. I have found that because of the greater openness or permeability of those portions of my nitrostarch stencil sheets which have been subjected to impact for the purpose of rendering them permeable to the ink, I am able to use inks of higher solid content than is possible with the duplicating inks used with nitrocellulose sheets, and I have further found that I can secure satisfactory impressions from my stencil sheet, with less pressure on the roller. Accordingly, by the use of my new stencil sheets of a nitrostarch base I am not only able to make use of inks containing less volatile solvent than the inks of the prior art, but I am able to make longer runs of duplicated matter before the stencil sheet becomes unusable, because of the reduced pressure that can be used on the roller in forcing the duplicating ink through the more open structure of the images produced in the preparation of my stencil sheets coated with nitrostarch composition.

The stencil sheets made in accordance with my present invention are accordingly superior to the nitrocellulose stencil sheets of the prior art in clearness of the reproduced matter, in the effective life of the stencil sheet, and in the ability to use not only a cheaper duplicating ink, but also an ink that shows quicker "setting" and reduced evaporation on the roller because of its increased solid content. Notwithstanding all of these advantages, I find that my nitrostarch coatings are just as impermeable to the duplicating inks at points where the stencil effect has not been intentionally produced, as the cellulose nitrate coated stencil sheets of the prior art.

I do not wish to be understood as claiming to obtain simultaneously under all conditions of use, all of the advantages of increased clearness of image, increased cheapness of ink and increased number of copies prepared from a stencil sheet before it becomes unusable, although under some conditions I do simultaneously obtain all of these advantages. In general, however, increased clearness of image is a characteristic that is always obtained with my new stencil sheets, as a result of the inherent characteristics of the relatively friable or disintegratable nitrostarch film as compared with the much tougher and much less friable cellulose nitrate coating of the prior art. If I employ with my nitrostarch stencil sheet the same ink that is employed with a nitrocellulose stencil sheet, I can use much lower pressure on my roller, and can accordingly obtain a much greater number of copies before the stencil sheet becomes weakened, marred, and no longer usable for high grade work. If, however, I increase the solid content of my ink, for the purpose of obtaining an ink which will not lose solvent as fast from the exposed portions of the roller, I find it desirable to use about the same pressure that is used on the roller of duplicating machines using nitrocellulose stencil sheets, and in this case I do not claim increased length of run with a stencil sheet of my new type, since the advantage of the use of the new sheet has been taken out in the use of a heavier ink, and this requires about the same roller pressure being

used with my more permeable stencil openings that would be used with a lighter ink and the less permeable stencil openings of a cellulose nitrate stencil sheet.

I do not claim any specific formulas for my nitrostarch stencil sheet coating compositions, as I have found that I may employ any of the formulas for nitrocellulose stencil coating compositions well known to those versed in the art, and I have found that the mere substitution of nitrostarch for nitrocellulose leads to the advantages and the improvements herein described. In general, I follow closely the teachings of the prior art, particularly as described in U. S. Patent 1,526,982 of February 17th, 1925, to Edward W. Hill, and I find that it is only necessary to substitute nitrostarch for nitrocellulose in any of the Hill or similar stencil compositions, to obtain the greatly improved results of increased openness and clearness of image, decreased roller pressure and the possibility of utilizing inks of less fluid nature than are required with the nitrocellulose sheets known up to the time of my present invention.

I do not find that the nitrogen content of the nitrostarch which I use is of any particular significance, and I have used nitrostarch ranging from 11.0% nitrogen to 13.0% nitrogen in conjunction with my present invention, with substantially similar results. I find nitrostarch of 13.0% nitrogen content is well adapted to use with the other components of stencil compositions, and is compatible with all of the other materials normally used in stencil manufacture, and is readily soluble in all of the solvents normally used in the preparation of nitrocellulose stencil sheets.

It will of course be understood that in the practice of my invention I use with nitrostarch any of the customary solvents (such as amyl acetate, for example), any of the customary pigments (such as carbon black, for example) any of the customary tempering agents (such as castor oil, for example), any of the customary setting agents (such as hydrogenated cotton-seed oil, for example) and any of the customary waxes (such as carnauba wax, for example) and in general I employ the same components, and in the same proportions, that are used in the preparation of the nitrocellulose class of stencil coating compositions of the prior art. Following the said patent to Hill, I may use, for instance, about 50% of the tempering agent on the weight of carbohydrate ester solution (in this case nitrostarch solution), a setting agent such as soya bean oil in amount to aid in setting the composition without making it sticky, and a limited proportion, say, 5 to 10% of a fatty or tallow-like material such as lard, cottolene, or Chinese vegetable tallow. For best results the combined weight of the tempering and setting agents and tallow-like or waxy material is not more than the weight of the original nitrostarch solution to which these ingredients are added.

I have discovered that the substitution of nitrostarch for nitrocellulose in the nitrocellulose stencil compositions of the prior art, leads to the very useful but unexpected result of providing stencils that are markedly superior in clarity of the duplicated matter, in the openness or porosity of the typed images, and in other respects, to the nitrocellulose stencil sheets known and widely used up to the time of my invention.

It will be evident that many changes may be made without departing from the scope of the invention as herein disclosed, and accordingly no limitations should be placed upon my invention, except such as are indicated in the appended claims.

I claim:

1. A stencil sheet, adapted to be converted into a stencil by the impact of type and the like thereon, comprising a fibrous base and a coating thereon, the coating including a type-impermeable, type-rupturable stencil composition of the carbohydrate ester class containing nitrostarch, a tempering agent, and a setting agent.

15 2. A stencil sheet, adapted to be converted

into a stencil by the impact of type and the like thereon, comprising a fibrous base and a coating thereon, the coating including a type-impermeable, type-rupturable stencil composition of the carbohydrate ester class containing nitrostarch, a tempering agent, and a setting agent.

3. A stencil sheet, adapted to be converted into a stencil by the impact of type and the like thereon, comprising a fibrous base and a coating thereon, the coating including a type-impermeable, type-rupturable stencil composition of the carbohydrate ester class containing nitrostarch, a tempering agent, and a waxy material.

WALTER O. SNELLING. 15